

Nov. 22, 1932.

E. L. CHAPPELL

1,888,961

## METHOD OF RECLAIMING PIPE

Filed Aug. 15, 1931



*Inventor:*  
EUGENE L. CHAPPELL,

by: *Alfred & Rauber*  
*his Attorneys.*

## UNITED STATES PATENT OFFICE

EUGENE L. CHAPPELL, OF PITTSBURGH, PENNSYLVANIA

## METHOD OF RECLAIMING PIPE

Application filed August 15, 1931. Serial No. 557,422.

This invention relates to a method of reclaiming corroded pipes and the like, and while not limited thereto relates more specifically to a method of reclaiming corroded pipe systems such as found in public buildings, dwellings and other large structures.

The object of this invention is to provide a method adapted to remove corrosion deposits from pipe systems and to provide a lining or coating of noncorrosive material on the interior of the system after the corrosion deposits have been removed.

Another object is the provision of a novel method of depositing a nonmetallic coating on pipes and pipe systems, such as a coating of cement or the like.

In the drawing:

Figure 1 is a diagrammatic showing of a piping system which has been divided into units, and has been equipped to carry out the method of this invention.

Figure 2 is an enlarged detail view showing the outlet end of one of the branch pipes.

Figure 3 is a detail view showing a form of outlet nozzle for use in the outlet hose sections.

Referring more particularly to the drawing, the numeral 2 designates a main header of a piping system which has a plurality of risers 3 leading therefrom. The risers 3 may be reduced in diameter intermediate their ends in accordance with plumbing practice, as between the points 15 and 16 of Figure 1. Each of the risers 3 is provided with a plurality of branch pipes 4, which may lead to sinks or the like throughout a building structure.

In carrying out the method of this application the piping system is treated in units, that is, each riser 3 and its branch lines 4 is assumed to be a unit, and is detached from the header 2 as shown at the right hand of Figure 1. This unit to be treated, after being detached from the head 2, has its lower end provided with a temporary connection 5 which leads to a tank or gun 6 (the purpose of which will be hereinafter described).

The tank or gun 6 has a removable top or cover portion 7, which is connected by a conduit 8 to a bank of fluid pressure storage

tanks 9 adapted to contain air or other gaseous fluid under pressure, the air or other gaseous fluid being delivered to the tanks 9 by a compressor 10 operated by a motor 12. The above fluid compressing unit is of ordinary and standard design and, therefore, will not be illustrated or described in detail.

The conduit 8 leading from the bank of tanks 9 to the vessel or gun 6 is provided with a main control valve 13 and a bleeder or relief valve 14.

After the above described apparatus has been connected to the lower end of the piping unit to be treated, the vessel or gun 6 will be filled with an abrasive material such as sand, iron filings, carborundum or any other suitable granular material and the compressed air or fluid under pressure will be turned into the vessel or gun 6 by opening the valve 13, thus blowing the abrasive material through the unit of the piping system to cut away and remove the corrosion deposits. It will be understood that any suitable sand blasting gun may be substituted for the gun 6. After the corrosion deposits have been removed, water or other liquid may be run through the unit of the piping system to remove any traces of the abrasive material and clear the surface of the pipe. This cleaning step may be omitted, if desired, and if used the liquid may be admitted either through the vessel or gun 6 or a temporary connection for the fluid may be substituted for the connection 5.

After the piping unit has been cleaned as above described, a quantity of cement grout will be placed in the gun or vessel to be forced through the cleaned unit. Prior to forcing the grout through the cleaned unit the risers 3 and each of the branch pipes 4 will be closed, with the exception of one or more of the branch pipes adjacent the end of the riser 3 farthest from the end at which the grout is to be admitted, which latter branch pipes are permitted to remain open as vents.

All of the branch pipes 4 are provided with sections of hose 4<sup>a</sup> at their outlet ends, which sections of hose carry nozzles 4<sup>b</sup> having restricted openings 4<sup>c</sup> therein of approximately 0.35 of the cross-sectional area of the branch pipes, and the branch pipes are adapted to be

closed by clamping these hose sections with squeezer tongs 20. The number of branch pipes adjacent the vented end of the riser 3 which are left open as vents are selected so that the combined restricted openings of their nozzles are adapted to equal approximately 0.35 of the cross-sectional area of the riser 3. Where the riser 3 is reduced, as between the points 15 and 16, vents, as at 15, are preferably left open to maintain the vent ratio throughout the riser.

Experience has shown that the most practical operating air or fluid pressure to use in carrying out this method is about 80 pounds gage pressure plus about one pound for every 15 foot of height when the coating material is being forced into the system. It has also been demonstrated that unless the pipes or units to be coated are restricted at their outer ends to approximately 0.35 of their cross-sectional 20 area the cement grout will not be properly distributed.

It should be understood that, if desired, various other fluid pressures may be used with proportionately greater or smaller outlet ports 4<sup>b</sup> in the nozzles 4<sup>b</sup> of the hose sections 4<sup>a</sup> to permit the proper flow of coating through the pipes.

With the unit vented as above described, the air or gaseous fluid under pressure will be admitted from the tanks 9 to the gun or vessel 6 by opening the valve 13, and the cement grout from the vessel or gun 6 will be blown upwardly through the riser 3 and outwardly through each of the branch pipes 4. This blowing of the grout will be continued until the air or gaseous fluid has escaped through the vents at the upper end of the unit, at which time the valve 40 13 will be closed and the valve 14 opened for bleeding or escape of the air or fluid from the vessel or gun 6 and the unit of piping. After the cement grout has been thus distributed throughout the unit the open or 45 vented branches 4 will be closed by applying the squeezer tongs 20 to the hose sections at the outer end of the branches, and the valve 13 will again be opened to admit air or gaseous fluid under pressure to the piping 50 unit, and each of the branch pipes 4 will then be opened momentarily to permit the fluid to blow therethrough to insure the clearing of each of said branch pipes. After each of the branch pipes has thus been blown, the 55 fluid pressure will again be taken off of the unit by closing the valve 13 and opening the valve 14. When the systems being coated includes elbows, bends, etc., it will then be permitted to stand without fluid pressure for a 60 time and then prior to the time the cement grout begins to set the vents and the valve 13 will again be opened and the valve 14 closed so as to again permit air or gaseous fluid to blow into the piping unit to insure the spreading 65 of any of the grout which may have run

back to form deposits at elbows or other points of the unit. This last blowing operation will only be momentary and will be stopped by closing the valve 13 and opening the valve 14. The unit will again be allowed 70 to rest until the grout has begun to set, at which time air or gaseous fluid under pressure may again be admitted to the unit by opening the vents and the valve 13 and closing the valve 14. This last blowing operation 75 also will be only momentary and serves to insure the removal of any deposits of the coating that may have accumulated at bends or in fittings of the unit.

If desired, fluid pressure may be applied to the unit after any or all of the above flowing operations and the squeezer tongs may be operated on any of the branch pipes 4 while said pressure is on the unit in order to insure the clearing of the branch pipes.

Experience has shown that blowing of the grout through a unit of the piping system can only be accomplished by the use of a high pressure and controlled rate of flow. By "high pressure" is meant a pressure of approximately 80 pounds gage pressure plus two pounds for each vertical height for lift and friction. As stated before, the unit is vented at or adjacent the end farthest away 90 from the point at which the grout enters and said vent or vents are equal to approximately 0.35 of the cross-sectional area of the pipe or pipes being coated. With a vent or vents of the above stated size, a fluid pressure of 80 pounds per square inch near the vents has 100 been found to be the most practical and to give the best spreading results when coating the pipe or pipes with cement grout.

It will, of course, be understood that while the above method has been described as applicable to piping systems, it is not limited to such use but may be applied to the coating of a single pipe or plurality of connected pipes, as desired. The coating may also be applied to pipes or piping systems which 110 are corroded or uncorroded, as desired. The only modification necessary when coating clean pipes or piping systems is the omission of the steps necessary for removing corrosion 115 deposits.

While I have illustrated my invention in connection with a schematic piping system and with a certain arrangement of apparatus, it will be understood that I do not wish to be limited thereto, since various forms of apparatus may be used in carrying out my invention and new forms of piping systems may be treated.

What I claim is:

1. The method of reclaiming corroded hollow metal articles, such as tanks, pipe and cylinders, which consists in blowing granular abrasive material through said article to remove the corrosion, then closing said article except for an inlet and vent, and then blowing

ing cement grout through said article, continuing the blowing until air passes through said vent, stopping the blowing, then blowing gaseous fluid under pressure through the article prior to the time the cement begins to set so as to spread any of the cement that has accumulated in deposits throughout the article being coated, and finally blowing gaseous fluid under pressure through the article as said cement begins to set, to finally spread any accumulated deposits of cement and clear the article.

2. The method of coating an assembled piping system which consists in separating said system into units consisting of one main feeder pipe and a series of branch pipes leading from said main feeder pipe, closing said main pipe and a sufficient number of the branch pipes to leave a vent area in the system of approximately 0.35 of the cross-sectional area of the main pipe, then blowing cement grout through said system, continuing the blowing until air passes through the vent, stopping the blowing and closing said vent, then applying gaseous fluid under pressure to the system and opening each of the several branch pipes and permitting the fluid to blow therethrough, removing the fluid pressure after blowing each of the said branch lines, again blowing gaseous fluid under pressure through said system just prior to the time said cement begins to set, for a short period, to spread the cement, again stopping said blowing of fluid under pressure until the cement begins to set, and then finally blowing fluid under pressure through the system after said cement has started to set to finally smooth the surface of the cement coating and clear any stoppages from the system unit.

3. The method of reclaiming a corroded piping system, which consists in separating said systems into units consisting of one main feeder pipe and a series of branch pipes leading from said main feeder pipe, blowing a granular abrasive material through said pipes to remove the corrosion, then closing said main pipe and sufficient of the branch pipes to leave a vent area in the system of approximately 0.35 of the cross-sectional area of the main pipe, then blowing cement grout through said system, continuing the blowing until air passes through the vent, stopping the blowing and closing said vent, then applying gaseous fluid under pressure to the system and opening each of the several branch pipes and permitting the fluid to blow therethrough, removing the fluid pressure after blowing each of the said branch lines, again blowing gaseous fluid under pressure through said system just prior to the time said cement begins to set, for a short period, to spread the cement, again stopping said blowing of fluid under pressure until cement begins to set, and then finally blowing fluid under pressure through the system after said cement has

started to set to finally smooth the surface of the cement coating and clear any stoppages from the system unit.

4. The method of coating hollow metal articles such as tanks, pipe and cylinders which consists in closing said article except for an inlet and vent, and then blowing semi-fluid, non-corrosive coating material through said vent, stopping the blowing, then blowing gaseous fluid under pressure through the article prior to the time the coating begins to set so as to spread any of the coating that has accumulated in deposits throughout the article being coated and finally blowing gaseous fluid under pressure through the article as said coating material begins to set to finally spread any accumulated deposits of material and clear the article.

5. The method of coating hollow metal articles such as tanks, pipe and cylinders which consists in closing said article except for an inlet and a vent, said vent being approximately 0.35 of the cross-sectional area of the article, and then blowing cement grout through the article, continuing the blowing until air passes through said vent, stopping the blowing, then blowing gaseous fluid under pressure through the article prior to the time the cement begins to set so as to spread any of the cement that has accumulated in deposits throughout the article being coated; and then finally blowing gaseous fluid under pressure through the article as said cement begins to set, to spread any accumulated deposits of cement and clear the article.

6. The method of coating an assembled piping system which consists in closing said system except for an inlet and vent, then blowing cement grout through said system, continuing the blowing until air passes through the vent, stopping the blowing and closing said vent, then applying gaseous fluid under pressure to the system and venting each individual line of the system and permitting the fluid to blow therethrough, removing the fluid pressure after blowing each of the individual lines of the system, again blowing gaseous fluid under pressure through said system just prior to the time said cement begins to set, for a short period, to spread the cement, again stopping said blowing of fluid under pressure until the cement begins to set, and then finally blowing fluid under pressure through the system after said cement has started to set to finally smooth the surface of the cement coating and clear any stoppages from the system.

7. The method of coating hollow metal articles such as tanks, pipe and cylinders which consists in closing said article except for an inlet and vent, said vent being of approximately 0.35 of the cross-sectional area of the article, and then blowing cement grout through said article from said inlet

at a pressure adapted to give a pressure of approximately eighty pounds per square inch adjacent the vent, continuing the blowing until air passes through said vent, stopping the blowing by blowing gaseous fluid through the article at substantially eighty pounds per square inch pressure prior to the time the cement begins to set so as to spread any of the cement that has accumulated in deposits throughout the article being coated, again stopping the blowing until said cement has begun to set, and finally blowing gaseous fluid under substantially eighty pounds per square inch pressure through the article after said cement has begun to set to finally spread any accumulated deposits of cement and clear the article.

In testimony whereof, I have hereunto set my hand.

EUGENE L. CHAPPELL.

20

25

30

35

40

45

50

55

60